# EUROPEAN PATENT SPECIFICATION

(11) **EP 2 049 631 B1**
(45) Date of publication and mention of the grant of the patent: **13.03.2013**
(21) Application number: 07840789.7
(22) Date of filing: 08.08.2007
(51) Int. Cl.: C10M 137/10, C10N 10/04, C10N 10/14, C10N 30/12, C10N 40/25

(54) **A LOW PHOSPHORUS LUBRICATING OIL COMPOSITION HAVING LEAD CORROSION CONTROL**
SCHMIERÖLZUSAMMENSETZUNG MIT GERINGEM PHOSPHORANTEIL UND BLEIKORROSIONSKONTROLLE
COMPOSITION D'HUILE LUBRIFIANTE DE FAIBLE TENEUR EN PHOSPHORE LIMITANT LA CORROSION DU PLOMB

(30) Priority: 09.08.2006 US 463532
(43) Date of publication of application: 22.04.2009
(73) Proprietor: Chevron Oronite Company LLC, San Ramon, CA 94583 (US)
(72) Inventor: BOFFA, Alexander B., Oakland, California 94618 (US)
(74) Representative: Nash, David Allan
(86) International application number: PCT/US2007/075507
(87) International publication number: WO 2008/021901

(56) References cited:
- EP-A1- 0 435 745
- EP-A1- 1 403 359
- US-A- 3 923 669
- US-A1- 2004 087 451
- US-A1- 2004 214 730
- US-B1- 6 596 672

## Description

The present invention is related, in part, to a lubricating oil composition. More particularly, the present invention relates to a low phosphorus lubricating oil composition employing a mixture of zinc dithiophosphates and wherein the lubricating oil composition has less than about 0.06 wt % total phosphorus content based on the total weight of the lubricating oil composition. The low phosphorus lubricating oil composition of the present invention is effective in lead corrosion control when used as a lubricating oil composition in internal combustion engines.

### BACKGROUND OF THE INVENTION

Emissions arising from automotive exhaust has been a problem for several decades and approaches for addressing this problem have included the use of unleaded fuel (to deal, in part, with lead pollution arising from leaded fuels), oxygenated fuel (to reduce hydrocarbon emissions), the use of catalytic converters (also to reduce hydrocarbon emissions), etc.

Catalytic converters are now universally employed with gasoline powered vehicles and the efficiency of these converters is directly related to the ability of the catalyst to effect conversion of unburnt or partially burnt hydrocarbons generated during combustion to carbon dioxide and water. One problem arising with the use of such converters is poisoning of the catalyst resulting in reduced catalyst efficiency. Since catalytic converters are intended for extended use, catalyst poisoning results in higher levels of atmospheric discharges of pollutants from internal combustion engines over prolonged periods of time.

In order to minimize such poisoning, the industry has set standards for both fuel and lubricant contents. For example, standards for fuels have included the use of unleaded gasoline in order to avoid lead poisoning of the catalyst as well as lead discharge into the environment. See, for example, Buckley, Ill, "*Long Chain Aliphatic Hydrocarbyl Amine Additives Having an Oxyalkylene Hydroxy Connecting Group",* U.S. Patent No. 4,975,096, issued December 4, 1990.

As to the lubricants, one additive family currently being addressed by industry standards is the phosphorus-containing additives such as zinc dithiophosphate wear inhibitors used lubricant compositions employed to lubricate internal combustion engines. Specifically, phosphorus-containing additives reach the catalytic converter as a result of, for example, exhaust gas recirculation and/or oil blow-by processes as well as other methods known in the art. See, for example, Beck, et al. "Impact of Oil-Derived Catalyst Poisons on FTP Performance of LEV Catalyst Systems"; SAE Technical Paper 972842 (1997) and Darr et al. "Effects of Oil-Derived Contaminants on Emissions from TWC-Equipped Vehicles", SAE 2000-01-1881 (2000). In any event, the phosphorus is known to accumulate in the catalytic converter, at active metal sites; thus reducing catalyst efficiency and effectively over time, poisoning the catalyst. As a result of the above, a new focus is to lower phosphorus in the lubricating oils. For example, the draft GF-4 specifications for lubricant compositions have proposed significantly lower phosphorus contents than heretofore employed.

A problem arises when the level of phosphorus is reduced in a lubricant composition containing an oil-soluble, phosphorus-containing, anti-wear compound in that there is a significant reduction in anti-wear performance arising from this diminution in phosphorus content. One well known class of antiwear additives are metal alkylphosphates, especially zinc dialkyl dithiophosphates, are generally employed in lubricating oils at phosphorous levels above 0.1 weight percent when used for wear control. At lower levels, it is not found to be an effective antiwear additive. For instance, as exemplified in U.S. Patent No. 6,696,393, issued February 24, 2004, lowering the level of phosphorus due to the presence of a metal dithiophosphate additive in a lubricant composition by one-half from 0.095 weight percent to 0.048 weight percent phosphorus results in about a seven-fold increase in engine wear.

Zinc dithiophosphates have either dialkyl or diaryl groups. Zinc dialkyl dithiophosphates are further subdivided into primary alkyl and secondary alkyl zinc dithiophosphates. Pentan-1-ol and 3-methylbutan-2-ol are illustrative of the primary and secondary alcohols used to prepare primary and secondary zinc dithiophosphates Different zinc dithiophosphate chemical types perform differently (See below).

### Performance Parameters of Zinc Dithiophosphate Types

| | Primary Alkyl | Secondary Alkyl | Aryl |
|---|---|---|---|
| Thermal Stability | | | |
| | Medium | Low | High |
| Antiwear Protection | | | |
| | Medium | High | Low |
| Hydrolytic Stability | | | |
| | Medium | High | Low |

Each type has important applications in modern additive packages. It is therefore important to have the right mix of zinc dithiophosphates in any given lubricating oil composition to provide adequate anti-wear performance and at the same time keeping the phosphorus levels, due to the presence of a metal dithiophosphate additive, below 0.1 wt % because phosphorus has a tendency to accumulate in the catalytic converter thus reducing catalyst efficiency, poisoning the catalyst.

EP 1 403 359 discloses a low ash lubricating oic composition inhibiting lead corrosion.

### SUMMARY OF THE INVENTION

As previously mentioned, the present invention is related, in part, to a lubricating oil composition. More particularly, the present invention relates to a low phosphorus lubricating oil composition employing a mixture of zinc dithiophosphates in a certain ratio and wherein the lubricating oil composition has less than about 0.06 wt % total phosphorus content, based on the total weight of the lubricating oil composition. The low phosphorus lubricating oil composition of the present invention is effective in lead corrosion control when used as a lubricating oil composition in internal combustion engines.

Accordingly, in its broadest aspect the present invention is related to a lubricating oil composition comprising a major amount of base oil of lubricating viscosity and a minor amount of at least 0.1 wt% to 1.5 wt% of a mixture of a zinc primary dialkyl dithiophosphate, a zinc secondary dialkyl dithiophosphate and a zinc diaryl dithiophosphate wherein the respective ratio, based on the phosphorus content, of the zinc primary dialkyl dithiophosphate to zinc secondary dialkyl dithiophosphate is from about 2:1 to about 1:2 and the ratio of the mixture of zinc primary dialkyl dithiophosphate and zinc secondary dialkyl dithiophosphate to zinc diaryl dithiophosphate is from about 6:1 to about 1:1 and wherein the total phosphorus content of the lubricating oil composition is less than about 0.06 wt %, based on the total weight of the lubricating oil composition.

The minor amount of the mixture of a zinc primary dialkyl dithiophosphate, a zinc secondary dialkyl dithiophosphate and a zinc diaryl dithiophosphate employed in the lubricating oil composition of the present invention is from about 0.1 wt % to about 1.5 wt %, preferably from about 0.3 wt % to about 1.2 wt % and more preferably about 0.5 wt % to about 1.0 wt %, based on the total weight of the lubricating oil composition.

The lubricating oil composition of the present invention will contain from about 0.05 wt % to about 1.2 wt % of a zinc primary dialkyl dithiophosphate, from about 0.05 wt % to about 1.2 wt % of a zinc secondary dialkyl dithiophosphate and from about 0.02 wt % to about 0.7 wt % of a zinc diaryl dithiophosphate, based on the total weight of the lubricating oil composition. Preferably, the lubricating oil composition of the present invention will contain from about 0.1 wt % to about 0.7 wt % of a zinc primary dialkyl dithiophosphate, from about 0.1 wt % to about 0.7 wt % of a zinc secondary dialkyl dithiophosphate and from about 0.05 wt % to about 0.5 wt % of a zinc diaryl dithiophosphate, based on the total weight of the lubricating oil composition. More preferably, the lubricating oil composition of the present invention will contain from about 0.2 wt % to about 0.5 wt % of a zinc primary dialkyl dithiophosphate, from about 0.2 wt % to about 0.5 wt % of a zinc secondary dialkyl dithiophosphate and from about 0.1 wt % to about 0.3 wt % of a zinc diaryl dithiophosphate, based on the total weight of the lubricating oil composition.

The primary alkyl group of the zinc primary dialkyl dithiophosphate has from about C₁ to about C₁₃ carbon atoms, preferably from about C₃ to about C₁₀ carbon atoms and more preferably, from about C₆ to about C₈ carbon atoms.

The secondary alkyl group of the zinc secondary dialkyl dithiophosphate has from about C₃ to about C₁₃ carbon atoms, preferably from about C₃ to about C₈ carbon atoms and more preferably, from about C₃ to about C₆ carbon atoms.

The aryl group of the zinc diaryl dithiophosphate has from about C₆ to about C₃₀ carbon atoms preferably from about C₆ to about C₂₄ carbon atoms and more preferably, from about C₆ to about C20 carbon atoms.

In a preferred embodiment, the respective ratio, based on the phosphorus content, of zinc primary dialkyl dithiophosphate to zinc secondary dialkyl dithiophosphate is from about 3:2 to about 2:3. More preferably, the ratio is about 1:1.

In a preferred embodiment, the respective ratio, based on the phosphorus content, of the mixture of zinc primary dialkyl dithiophosphate and zinc secondary dialkyl dithiophosphate to zinc diaryl dithiophosphate is from about 4:1 to about 1:1. More preferably, the ratio is bout 2:1.

In an especially preferred embodiment, the respective ratio, based on the phosphorus content, of the mixture of zinc primary dialkyl dithiophosphate to zinc secondary dialkyl dithiophosphate to zinc diaryl dithiophosphate is 1:1:1.

In another embodiment, the total phosphorus content in the lubricating oil composition of the present invention is preferably less than about 0.05 wt %, more preferably, based on the total weight of the lubricating oil composition.

In still another embodiment, the sulfur content in the lubricating oil composition of the present invention is less than about 0.5 wt % and, preferably, less than about 0.2 wt %, based on the total weight of the lubricating oil composition and the total sulfated ash contest in the lubricating oil composition of the present invention is less than about 1.2 wt %, preferably, less than about 1.0 wt %, and more preferably less than about 0.8 wt %, based on the total weight of the lubricating oil composition.

In one of its method aspects, the present invention further relates to a method for improving lead corrosion. The method involves operating an internal combustion engine with a lubricating oil composition comprising a major amount of base oil of lubricating viscosity and a minor amount of a mixture of a zinc primary dialkyl dithiophosphate, a zinc secondary dialkyl dithiophosphate and a zinc diaryl dithiophosphate wherein the respective ratio, based on the phosphorus content, of the zinc primary dialkyl dithiophosphate to zinc secondary dialkyl dithiophosphate is from about 2:1 to about 1:2 and the ratio of the mixture of zinc primary dialkyl dithiophosphate and zinc secondary dialkyl dithiophosphate to zinc diaryl dithiophosphate is from about 6:1 to about 1:1 and wherein the total phosphorus content of the lubricating oil composition is less than about 0.06 wt %, based on the total weight of the lubricating oil composition.

Among other factors, the present invention provides a low phosphorus lubricating oil composition containing a mixture of zinc dithiophosphates in a certain ratio surprisingly yields improved lead corrosion. The mixture of zinc dithiophospates contains a zinc primary dialkyl dithiophosphate, a zinc secondary dialkyl dithiophosphate and a zinc diaryl dithiophosphate. The synergistic combination of mixed zinc dithiophosphates wherein the respective ratio, based on the phosphorus content, of the zinc primary dialkyl dithiophosphate to zinc secondary dialkyl dithiophosphate is from about 2:1 to about 1:2 and the ratio of the mixture of zinc primary dialkyl dithiophosphate and zinc secondary dialkyl dithiophosphate to zinc diaryl dithiophosphate is from about 6:1 to about 1:1 when used in a lubricating oil composition having a total phosphorus content less than about 0.06 wt %, based on the total weight of the lubricating oil composition, greatly reduces lead corrosion when used to lubricate internal combustion engines.

### DETAILED DESCRIPTION OF THE INVENTION

The present invention is related, in part, to a lubricating oil composition. More particularly, the present invention relates to a low phosphorus lubricating oil composition employing a mixture of zinc dithiophosphates containing a zinc primary dialkyl dithiophosphate, a zinc secondary dialkyl dithiophosphate and a zinc diaryl dithiophosphate wherein the respective ratio, based on the phosphorus content, of the zinc primary dialkyl dithiophosphate to zinc secondary dialkyl dithiophosphate is from about 2:1 to about 1:2 and the ratio of the mixture of zinc primary dialkyl dithiophosphate and zinc secondary dialkyl dithiophosphate to zinc diaryl dithiophosphate is from about 6:1 to about 1:1 and wherein the lubricating oil composition has less than about 0.06 wt % total phosphorus content, based on the total weight of the lubricating oil composition. The low phosphorus lubricating oil composition of the present invention is effective in lead corrosion control when used as a lubricating oil in internal combustion engines.

Each of these components in the claimed composition will be described in detail herein. However, prior to such a description, the following terms will first be defined.

The term "alkyl" refers to both straight- and branched-chain alkyl groups.

The term "aryl" refers to a substituted or unsubstituted aromatic group, such as the phenyl, tolyl, xylyl, ethylphenyl and cumenyl groups.

The term "low phosphorus" refers to the phosphorus content of the lubricating oil composition of the present invention. The phosphorus content is in the range of about 0.005 weight percent to about 0.06 weight percent based on the total weight of the lubricating oil composition.

The term "total phosphorus" refers to the total amount of phosphorus in the lubricant composition regardless of whether such phosphorus is present as part of an oil-soluble, phosphorus-containing, anti-wear compound or in the form of a contaminant in the lubricant composition such as residual phosphorus remaining due to the presence of P₂S₅ used to prepare metal dihydrocarbyl dithiophosphates. In either event, the amount of phosphorus permitted in the lubricant composition is independent of source. Preferably, however, the phosphorus is part of a lubricant additive.

Unless otherwise specified, all percentages are in weight percent.

### The Zinc Dithiophosphate Compound

The lubricating oil composition of the present invention will employ, in part, a mixture of zinc dithiophosphates. The zinc dithiophosphates are independently characterized by formula I: wherein each R is independently a group containing from about 1 to about 30 carbon atoms.

The R groups in the dithiophosphate can independently be about C₁ to about C₁₃ primary alkyl, about C₃ to about C₁₃ secondary alkyl and about C₆ to about C₃₀ aryl group. Preferably, the R groups in the dithiophosphate can independently be about C₃ to about C₁₀ primary alkyl, about C₃ to about C₈ secondary alkyl, and about C₆ to about C₂₄ aryl group. More preferably, the R groups in the dithiophosphate can independently be about C₆ to about C₈ primary alkyl, about C₃ to about C₆ secondary alkyl, and about C₆ to about C₂₀ aryl group. The R groups may be a substantially hydrocarbon group. By "substantially hydrocarbon" is meant hydrocarbons that contain substituent groups such as ether, ester, nitro, or halogen which do not materially affect the hydrocarbon character of the group.

The R group of the zinc dithiophosphate may be derived, for example, from a primary alcohol such as methanol, ethanol, propanol, butanol, pentanol, hexanol, heptanol, octanol, nonanol, decanol, dodecanol, octadecanol, propenol, butenol, 2-ethylhexanol; a secondary alcohol such as isopropyl alcohol, secondary butyl alcohol, isobutanol, 3-methylbutan-2-ol, 2-pentanol, 4-methyl-2-pentanol, 2-hexanol, 3-hexanol, amyl alcohol; an aryl alcohol such as phenol, substituted phenol (particularly alkylphenol such as butylphenol, octylphenol, nonylphenol, dodecylphenol), disubstituted phenol.

Preferably the R group will be independently a primary alkyl, a secondary alkyl or an aryl group.

For the present invention it is contemplated that the mixture of a zinc primary dialkyl dithiophosphate, a zinc secondary dialkyl dithiophosphate and a zinc diaryl dithiophosphate will be in a respective ratio, based on the phosphorus content, in the Lubricating oil composition of the present invention. The ratio of zinc primary dialkyl dithiophosphate to zinc secondary dialkyl dithiophosphate will be from about 2:1 to about 1:2 and the ratio of the mixture of zinc primary dialkyl dithiophosphate and zinc secondary dialkyl dithiophosphate to zinc diaryl dithiophosphate is from about 6:1 to about 1:1. Preferably, the respective patio, based on the phosphorus content, of zinc primary dialkyl dithiophosphate to zinc secondary dialkyl dithiophosphate is a range from about 3:2 to about 2:3, more preferably about 1:1. Preferably, the respective ratio, based on the phosphorus content, of the mixture of zinc primary dialkyl dithiophosphate and zinc secondary dialkyl dithiophosphate to zinc diaryl dithiophosphate is a range from about 4:1 to about 1:1, more preferably about 2:1. Most preferably, the respective ratio, based on the phosphorus content, of the mixture of zinc primary dialkyl dithiophosphate to zinc secondary dialkyl dithiophosphate to zinc diaryl dithiophosphate is 1:1:1.

Many of the zinc dithiophosphates useful in the present invention are available commercially. However, zinc dithiophosphates are widely known in the art and a skilled artisan can readily synthesize such compounds for the purpose of the present invention. Typically, zinc dithiophosphates can be made by initial reaction of phosphorous pentasulfide and an alcohol or phenol or mixtures of alcohols and/or phenols such as those illustrated above for the R group. The reaction involves four moles of the alcohol or phenol per mole of phosphorous pentasulfide, and may be carried out within the temperature range from about 50°C to about 200°C. Thus, the preparation of O,O-di-n-hexyl phosphorodithioic acid, for example, involves the reaction of phosphorous pentasulfide, with four moles of n-hexyl alcohol at about 100°C for about two hours. Hydrogen sulfide is liberated and the residue is phosphorodithioic acid. The preparation of the metal salt of this acid may be effected by reaction with either zinc oxide or zinc hydroxide to yield the zinc dithiophosphate. Simply mixing and heating these two reactants is sufficient to cause the reaction to take place and the resulting product is sufficiently pure for the purposes of the present invention.

Patents describing the synthesis of such zinc dithiophosphates include U.S. Patent Nos. 2,680,123; 3,000,822; 3,151,075; 3,385,791; 4,377,527; 4,495,075 arid 4,778,906. Each of these patents is incorporated herein by reference in their entirety.

### The Lubricating Oil Composition

The mixture of zinc dithiophosphates of the present invention is typically added to a base oil in sufficient amounts to provide lead corrosion control in internal combustion engines. Generally, the lubricating oil composition of the present invention will contain a major amount of base oil of fabricating viscosity and a minor amount of the mixture of zinc dithiophosphates of the present invention.

### Bas Oil of Lubricating Viscosity

Base oil as used herein is defined as a base stock or blend of base stocks which is a lubricant component that is produced by each manufacturer to the same specifications (independent of feed source or manufacturer's location); that meets the same manufacturer's specification; and that is identified by a unique formula, product identification number, or both. Base stocks may be manufactured using a variety of different processes including but not limited to distillation, solvent refining, hydrogen processing, oligomerization, esterification, and redefining.

Rerefined stock shall be substantially free from materials introduced through manufacturing, contamination, or previous use. The base oil of this invention may be any natural or synthetic lubricating base oil fraction particularly those having a kinematic viscosity at 100° Centigrade, (°C) and about 4 centistokes (cSt) to about 20 cSt. Hydrocarbon synthetic oils may include, for example, oils prepared from the polymerization of ethylene, polyalphaolefin or PAO, or from hydrocarbon synthesis procedures using carbon monoxide and hydrogen gasses such as in a Fisher-Tropsch process. A preferred base oil is one that comprises little, if any, heavy fraction; e.g., little, if any, lube oil fraction of viscosity about 20 cSt or higher at about 100°C Oils used as the base oil will be selected or blended depending on the desired end use and the additives in the finished oil to give the desired grade of engine oil, e.g. a lubricating oil composition having an SAE Viscosity Grade of 0W, 0W-20, 0W-30, 0W-40, 0W-50, 0W-60, 5W, 5W-20, 5W-30, 5W-40, 5W-50, 5W-60, 10W, 10W-20, 10W-30, 10W-40, 10W-50, 15W, 15W-20, 15W-30, or 15W-40.

The base oil may be derived from natural lubricating oils, synthetic lubricating oils or mixtures thereof. Suitable base oil includes base stocks obtained by isomerization of synthetic wax and stack wax, as well as hydrocrackate base stocks produced by hydrocracking (rather than solvent extracting) the aromatic and polar components of the crude. Suitable base oils include those in all API categorizes I, II, III, IV and V as defined in API Publication 1509, 14th Edition, Addendum I, December 1998. Saturates levels and viscosity indices, for Group I, II and 111 base oils are listed in Table I. Group IV base oils are polyalphaolefins (PAO). Group V base oils include all other base oils not included in Group I, II, III, or IV. Group III base oils are preferred.

**TABLE I.**

| SATURATES, SULFUR AND VISCOSITY INDEX OF GROUP I, II, III, IV AND V BASE STOCKS | | |
|---|---|---|
| Group | Saturates (As determined by ASTM D2007) | Viscosity Index |
| | Sulfur (As determined by ASTM D2270) | (As determined by ASTM D4294, ASTM D4297 or ASTM D3120) |
| I. | Less than 90 % saturates and/or Greater than to 0.03 % sulfur | Greater than or equal to 80 and less than 120 |
| II. | Greater than or equal to 9.0 % saturates and less than or equal to 0.03 % sulfur | Greater than or equal to 80 and les than 120 |
| III | Greater than or equal to 90 % saturates and less than or equal to 0.03% sulfur | Greater than or equal to 120 |
| IV | All Polyalphaolefins (PAOs) | |
| V | All others not included in Groups I, II, III, or IV | |

Natural lubricating oils may include animal oils, vegetable oils (e.g., rapeseed oils, castor oils and lard oil), petroleum oils, mineral oils, and oils derived from coal or shale.

Synthetic oils may include hydrocarbon oils and halo-substituted hydrocarbon oils such as polymerized and inter-polymerized olefins, alkylbenzenes, polyphenyls, alkylated diphenyl ethers, alkylated diphenyl sulfides, as well as their derivatives, analogues and homologues thereof, and the like. Synthetic lubricating oils also include alkylene oxide polymers, interpolymers, copolymers and derivatives thereof wherein the terminal hydroxyl groups have been modified by esterification, etherification, etc. Another suitable class of synthetic lubricating oils comprises the esters of dicarboxylic acids with a variety of alcohols. Esters useful as synthetic oils also include those made from about C₅ to about C₁₂ monocarboxylic acids and polyols and polyol ethers Tri-alkyl phosphate ester oils such as those exemplified by tri-n-butyl phosphate and tri-iso-butyl phosphate are also suitable for use as base oils.

Silicon-based oils (such as the polyalkyl-, polyaryl-, polyalkoxy-, or polyaryloxysiloxane oils and silicate oils) comprise another useful class of synthetic lubricating oils. Other synthetic lubricating oils include liquid esters of phosphorus-containing acids, polymeric tetrahydrofurans, polyalphaolefins, and the like.

The base oil may be derived from unrefined, refined, rerefined oils; or mixtures thereof. Unrefined oils are obtained directly from a natural source or synthetic source (e.g., coal, shale, or tar sand bitumen) without further purification or treatment: Examples of unrefined oils include a shale oil obtained directly from a retorting operation, a petroleum oil obtained directly from distillation, or an ester oil obtained directly from an esterification process, each of which may then be used without further treatment. Refined oils are similar to the unrefined oils except that refined oils have been treated in one or more purification steps to improve one or more properties. Suitable purification techniques include distillation, hydrocracking, hydrotreating, dewaxing, solvent extraction, acid or base extraction, filtration, and percolation, all of which are known to those skilled in the art Rerefined oils are obtained by treating used oils in processes similar to those used to obtain the refined oils. These rerefined oils are also known as reclaimed or reprocessed oils and often are additionally processed by techniques for removal of spent additives and oil breakdown products.

Base oil derived from the hydroisomerization of wax may also be used, either alone or in combination with the aforesaid natural and/or synthetic base oil.

Such wax isomerate oil is produced by the hydroisomerization of natural or synthetic waxes or mixtures thereof over a hydroisomerization catalyst.

It is preferred to use a major amount of base oil in the lubricating oil composition of the present invention. A major amount of base oil as defined herein comprises about 40 wt % or more. Preferred amount of base oil comprise about 40 wt % to about 97 wt %, preferably greater than about 50 wt % to about 97 wt %, more preferably about 60 wt % to about 97 wt % and most preferably about 80 wt % to about 95 wt % of the lubricating oil composition. (when weight percent is used herein, it is referring to weight percent of the lubricating oil unless otherwise specified.)

The amount of the mixture of zinc dithiophosphates employed in the lubricating oil composition of the present invention will be in a minor amount compared to the base oil of lubricating viscosity. Generally, it will be in an amount from about 0.1 wt % to about 1.5 wt%, preferably from about 03.3 wt % to about 1.2 wt % and more preferably from about 0.5 wt % to about 1.0 wt %, based on the total weight of the lubricating oil composition.

The lubricating oil composition of the present invention will contain from about 0.05 wt % to about 1.2 wt %, preferably from about 0.1 wt % to about 0.7 wt %, and more preferably from about 0.2 wt % to about 0.5 wt % of a zinc primary dialkyl dithiophosphate, based on the total weight of the lubricating oil composition.

The lubricating oil composition of the present invention will contain from about 0.05 wt % to about 1.2 wt %, preferably from about 0.1 wt % to about 0.7 wt %, and more preferably from about 0.2 wt % to about 0.5 wt % of a zinc secondary dialkyl dithiophosphate, based on the total weight of the lubricating oil composition.

The lubricating oil composition of the present invention will contain from about 0.02 wt % to about 0.7 wt %, preferably from about 0.05 wt % to about 0.5 wt %, and more preferably from about 0.1 wt % to about 0.3 wt % of a zinc primary diaryl dithiophosphate, based on the total weight of the lubricating oil composition.

In a preferred embodiment, the lubricating oil composition of the present invention will have a phosphorus content preferably less than about 0.05 wt %, based on the total weight of the lubricating oil composition.

In another embodiment, the lubricating oil composition of the present invention will further have a sulfur content less than about 0.5 wt % and, preferably less than about 0 2 wt %, based on the total weight of the lubricating oil composition and the total sulfated ash content in the lubricating oil composition of the present invention is less than about 1.2 wt %, preferably, less than about 1.0 wt %, and more preferably less than about 0.8 wt %, based on the total weight of the lubricating oil composition.

### Other Additive Components

The following additive components are examples of components that can be favorably employed in combination with the lubricating additive of the present invention. These examples of additives are provided to illustrate the present invention, but they are not intended to limit it.
(A) Detergents are additives designed to hold the acid-neutralizing compounds in solution the the oil. They are usually alkaline and react with the strong acids (sulfuric and nitric) which form during the combustion of the fuel and which would cause corrosion to the engine parts if left unchecked. Examples are carboxylates, sulfurized or unsulfurized alkyl or alkenyl phenates, alkyl or alkenyl aromatic sulfonates, sulfurized or unsulfurized metal salts of multi-hydroxy alkyl or alkenyl aromatic compounds, alkyl or alkenyl hydroxy aromatic sulfonates, sulfurized or unsulfurized alkyl or alkenyl naphthenates, metal salts of alkanoic acids, metal salts of an alkyl or alkenyl multiacids and chemical and physical mixtures thereof.
(B) Dispersants are additives that keep .soot and combustion products in suspension in the body of the oil and therefore prevent deposition as sludge or lacquer Typically, the ashless dispersants are nitrogen-containing dispersants formed by reacting alkenyl succinic acid anhydride with an amine. Examples are alkenyl succinimides, alkenyl succinimides modified with other organic compounds, e.g., ethylene carbonating post-treatment and alkenyl succinimides modified with boric acid, polysuccinimides, alkenyl succinic ester.
(C) Oxidation Inhibitors:
   1) Phenol type (phenolic) oxidation inhibitors: 4,4'-methylenebis (2,6-di-tertbutylphenol), 4,4'-bis(2,6-di-tert-butylphenol), 4,4'-bis(2-methyl-6-tertbutylphenol), 2,2'-methylenebis(4-methyl-6-tert-butyl-phenol), 4,4'-butyldienebis(3-methyl-6-tert-butylphenol), 4,4'-isopropylidenebis(2,6-di-tertbutylphenol), 2,2'-methylenebis(4-methyl-6-nonylphenol), 2,2'-isobutyldiene-bis(4,6-dimethylphenol), 2,2'-methylenebis(4-methyl-6-cyclohexylphenol), 2,6-di-tert-butyl-4-methylphenol, 2,6-di-tert-butyl-4-ethylphenol, 2,4-dimethyl-6-tert-butyl-phenol, 2,6-di-tert-α-dimethylamino-p-cresol, 2,6-di-tert-4(N,N' dimethylaminomethylphenol), 4,4'-thiobis(2-methyl-6-tert-butylphenol), 2,2'-thiobis(4-methyl-6-tert-butylphenol), bis(3-methyl-4-hydroxy-5-tert-butylbenzyl)-sulfide and bis (3,5-di-tert-butyl-4-hydroxybenzyl),
   2) Diphenylamine type oxidation inhibitor: alkylated diphenylamine, phenyl-α-naphthylamine and alkylated α-naphthylamine.
   3) Other types: metal dithiocarbamate (e.g., zinc dithiocarbamate) and methylenebis(dibutyldithiocarbamate).
(D) Rust Inhibitors (Anti-rust agents):
   1) Nonionic polyoxyethylene surface active agents: polyoxyethylene lauryl ether, polyoxyethylene higher alcohol ether, polyoxyethylene nonylphenyl ether, polyoxyethylene octylphenyl ether, polyoxyethylene octyl stearyl ether, polyoxyethylene oleyl ether, polyoxyethylene sorbitol monostearate, polyoxyethylene sorbitol mono-oleate and polyethylene glycol monooleate.
   2) Other compounds: stearic acid and other fatty acids, dicarboxylic acids, metal soaps, fatty acid amine salts, metal salts of heavy sulfonic acid, partial carboxylic acid ester of polyhydric alcohol and phosphoric ester.
(E) Demulsifiers: addition product of alkylphenol and ethyleneoxide, polyoxyethylene alkyl ether and polyoxyethylene sorbitane ester.
(F) Extreme pressure agents (EP agents): sulfurized oils, diphenyl sulfide, methyl trichlorostearate, chlorinated naphthalene, benzyl iodide, fluoroalkylpolysiloxane and lead naphthenate.
(G) Friction modifiers: fatty alcohol, fatty acid, amine, borated ester and other esters.
(H) Multifunctional additives: sulfurized oxymolybdenum dithiocarbamate, sulfurized oxymolybdenum organo phosphorodithioate, oxymolybdenum monoglyceride, oxymolybdenum diethylate amide, amine-molybdenum complex compound and sulfur-containing molybdenum complex compound
(I) Viscosity Index Improvers (VII): polymethacrylate type polymers, ethylenepropylene copolymers, styrene-isoprene copolymers, hydrogenated styrene-isoprene copolymers, hydrogenated star-branched polyisoprene, polyisobutylene, hydrogenated star-branched styrene-isoprene copolymer and dispersant type viscosity index improvers.
(J) Pour point depressants: polymethyl methacrylates, alkylmethacrylates and dialkyl fumarate-vinyl acetate copolymers.
(K) Foam Inhibitors: alkyl methacrylate polymers and dimethyl silicone polymers.

### EXAMPLES

The present invention will be further illustrated by the following examples, which set forth particularly advantageous method ennbodiments. While the Examples are provided to illustrate the present invention, they are not intended to limit it.

### Example 1

The low phosphorus lubricating oil composition of the present invention was prepared by blending a 0.78 wt % mixture of zinc bis(O,O'-di-(2-ethyl-1-hexyl) dithiophosphate (0.24 wt%, primary), zinc bis(O,O'-di-(2-butyl/4-methyl-2-pentyl) dithiophosphate (0.15 wt %, secondary) and zinc bis(O,O'-di-(dodecylphenyl) dithiophosphate (0.39 wt %, aryl) with a Group II base oil of lubricating viscosity. The ratio of zinc bis(O,O'-di(2-ethyl-1-hexyl) dithiophosphate to zinc bis(O,O'-di-(2-butyl/4-methy)-2-pentyl) dithiophosphate was about 1:1, based on the phosphorus content. The ratio of the mixture of zinc bis(O,O'-di(2-ethyl-1-hexyl) dithiophosphate and zinc bis(O,O'-di-(2-butyl/4-methyl-2-pentyl) dithiophosphate to zinc bis(O,O'-di-(dodecylphenyl) dithiophosphate was about 2:1, based on the phosphorus content. The resulting ratio of the three-way mixture of zinc bis(O,O'-di(2-ethyl-1-hexyl) dithiophosphate to zinc bis(O,O'-di'-(2-butyl/4-methyl-2-pentyl) dithiophosphate to zinc bis(O,O'-di(dodecylphenyl) dithiophosphate was 1:1:1, based on the phosphorus content. The wt % of phosphorus in the prepared lubricating oil composition was less than about 0.06 wt % based on the total weight of the lubricating oil composition. Further, the sulfur content and sulfated ash content were 0.2 wt% and 0.8 wt%, respectively, based on the total weight of the lubricating oil composition. The wt % balance of the lubricating oil composition containing a 1200 molecular weight (MW) isobutylene bis-succinimide dispersant, a 2300 MW isobutylene bis-succinimide dispersant, a neutral sulfonate detergent, an overbased calcium phenate, a molybdenum oxidation inhibitor, diphenylamine oxidation inhibitor, a phenolic oxidation inhibitor, anti-foam agent, pour point depressant and a viscosity index improver to complete the 100 wt % lubricating oil composition.

### Comparative Example A

Comparative Example A was prepared according to Example 1 except only about 1.16 wt % aryl zinc bis(O,O'-di-(dodecylphenyl) dithiophosphate was added, instead of the mixture of zinc bis(O,O'-di-(2-ethyl-1-hexyl) dithiophosphate, zinc bis(O,O'-di-(2-butyl/4-methyl-2-pentyl) dithiophosphate and zinc bis(O,O'-di-(dodecylphenyl) dithiophosphate.

### Comparative Example B

Comparative Example B was prepared according to Example 1 except only about 0.46 wt % zinc bis(O,O'-di-(2-butyl-4-methyl-2-pentyl) dithiophosphate was added, instead of the mixture of zinc-bis(O,O'-di-(2-ethyl-1-hexyl) dithiophosphate, zinc bis(O,O'-di-(2-butyl/4-methyl-2-pentyl) dithiophosphate and zinc bis(O,O'-di-(dodecylphenyl) dithiophosphate.

### Comparative Example C

Comparative Example C was prepared according to Example 1 except only about 0.71 wt % zinc bis(O,O'-di-(2-ethyl-1-hexyl) dithiophosphate was added, instead of the mixture of zinc bis(O,O'-di-(2-ethyl-1-hexyl) dithiophosphate, zinc bis(O,O'-di-(2-butyl/4-methyl-2-pentyl) dithiophosphate and zinc bis(O,O'-di-(dodecylphenyl) dithiophosphate.

### Comparative Example D

Comparative Example D was prepared according to Example 1 except about 0.81 wt % of a mixture of zinc bis (O,O'-di-(2-butyl/4-methyl-2-pentyl) dithiophosphate and zinc bis (O,O'-di-(dodecylphenyl) dithiophosphate in about a 1:1 ratio were added, instead of the mixture of zinc bis(O,O-di-(2-ethyl-1-hexyl) dithiophosphate zinc bis(O,O'-di-(2-butyl/4-methyl-2-pentyl) dithiophosphate and zinc bis (O,O'-di-(dodecylphenyl) dithiophosphate.

### Comparative Example E

Comparative Example E was prepared according to Example 1 except about 0.94 wt % of a mixture of zinc bis(O,O'-di-(2-ethyl-1-hexyl) dithiophosphate and zinc bis(O,O'-di-(dodecylphenyl) dithiophosphate in about a 1:1 ratio were added, instead of the mixture of zinc bis(O,O'-di-(2-ethyl-1-hexyl) dithiophosphate, zinc bis (O,O'-di-(2-butyl/4-methyl-2-pentyl) dithiophosphate and zinc bis(O,O'-di-(dodecylphenyl) dithiophosphate.

### Comparative Example F

Comparative Example F was prepared according to Example 1 except about 0.59 wt% of a mixture of zinc bis (O,O'-di-(2-ethyl-1-hexyl) dithiophosphate and zinc bis(O,O'-di-(2-butyl/4-methyl-2-pentyl) dithiophosphate in about a 1:1 ratio were added, instead of the mixture of zinc bis(O,O'-di-(2-ethyl-1-hexyl) dithiophosphate, zinc bis(O,O'-di-(2-butyl/4-methyl-2-pentyl) dithiophosphate and zinc bis(O,O'-di-(dodecylphenyl) dithiophosphate.

Each formulation according to Example 1 and Comparative Example A-F were tested for lead corrosion using the High Temperature Corrosion Bench Test (HTCBT)(ASTM D6594) which is an industry standard bench test to measure corrosion performance of a motor oil. Briefly, four metal specimens of copper, lead, tin, and phosphor bronze are immersed in a measured amount of engine oil. The oil, at an elevated temperature, is blown with air for a period of time. When the test is completed, the lead specimen and the stressed oil are examined to detect corrosion and corrosion products, respectively. A reference oil is tested with:each group of tests to verify test acceptability.

The test results are summarized in Table II.

**Table II. HTCBT Results**

| | Example 1 | Comparative Examples | | | | | |
|---|---|---|---|---|---|---|---|
| | | A | B | C | D | E | F |
| Lead, ppm | 48.4 | 113.4 | 93.4 | 305 | 64.6 | 87.3 | 99.4 |

These results demonstrate that the low phosphorus lubricating oil composition of the present invention (Example 1) containing a mixture of zinc primary dialkyl dithiophosphate, zinc secondary dialkyl dithiophosphate and zinc diaryl dithiophosphate in a 1:1:1 ratio, and wherein the phosphorus content of the lubricating oil composition is less than 0.06 wt%, provides excellent lead corrosion performance when compared to the comparative examples not having a mixture of all three dithiophosphates. The amount of lead corrosion is significantly reduced by the lubricating oil composition of the present invention.

## Claims

1. A lubricating oil composition comprising a major amount of base oil of lubricating viscosity and a minor amount of at least 0.1 wt.% to 1.5 wt.% of a mixture of a zinc primary dialkyl dithiophosphate, a zinc secondary dialkyl dithiophosphate and a zinc diaryl dithiophosphate wherein the respective ratio, based on the phosphorus content, of the zinc primary dialkyl dithiophosphate to zinc secondary dialkyl dithiophosphate is from 2:1 to 1:2 and the ratio of the mixture of zinc primary dialkyl dithiophosphate and zinc secondary dialkyl dithiophosphate to zinc diaryl dithiophosphate is from 6:1 to 1:1 and wherein the lubricating oil composition has less than 0.06 wt % total phosphorus content, based on the total weight of the lubricating oil composition.

2. The lubricating oil composition according to Claim 1, wherein the minor amount of the mixture of zinc primary dialkyl dithiophosphate, zinc secondary dialkyl dithiophosphate and zinc diaryl dithiophosphate is from 0.3 wt % to 1.2 wt %, based on the total weight of the lubricating oil composition; or wherein the minor amount of the mixture of zinc primary dialkyl dithiophosphate, zinc secondary dialkyl dithiophosphate and zinc diaryl dithiophosphate is from 0.5 wt % to 1.0 wt %, based on the total weight of the lubricating oil composition.

3. The lubricating oil composition according to Claim 1, wherein the mixture contains from 0.05 wt % to 1.2 wt % zinc primary dialkyl dithiophosphate, from 0.05 wt % to 1.2 wt % zinc secondary dialkyl dithiophosphate and from 0.02 wt % to 0.7 wt % zinc diaryl dithiophosphate, based on the total weight of the lubricating oil composition; or wherein the mixture contains from 0.1 wt % to 0.7 wt % zinc primary dialkyl dithiophosphate, from 0.1 wt % to 0.7 wt % zinc secondary dialkyl dithiophosphate and from 0.05 wt % to 0.5 wt % zinc diaryl dithiophosphate, based on the total weight of the lubricating oil composition; or wherein the mixture contains from 0.2 wt % to 0.5 wt % zinc primary dialkyl dithiophosphate, from 0.2 wt % to 0.5 wt % zinc secondary dialkyl dithiophosphate and from 0.1 wt % to 0.3 wt % zinc diaryl dithiophosphate, based on the total weight of the lubricating oil composition.

4. The lubricating oil composition according to Claim 1, wherein the primary alkyl group of the zinc primary dialkyl dithiophosphate has from C₁ to C₁₃ carbon atoms; or wherein the primary alkyl group of the zinc primary dialkyl dithiophosphate has from C₃ to C₁₀ carbon atoms; or wherein the primary alkyl group of the zinc primary dialkyl dithiophosphate has from C₆ to C₈ carbon atoms.

5. The lubricating oil composition according to Claim 1, wherein the secondary alkyl group of the zinc secondary dialkyl dithiophosphate has from C₃ to C₁₃ carbon atoms; or wherein the secondary alkyl group of the zinc secondary dialkyl dithiophosphate has from C₃ to C₈ carbon atoms; or wherein the secondary alkyl group of the zinc secondary dialkyl dithiophosphate has from C₃ to C₆ carbon atoms.

6. The lubricating oil composition according to Claim 1, wherein the aryl group of the zinc diaryl dithiophosphate has from C₆ to C₃₀ carbon atoms; or wherein the aryl group of the zinc diaryl dithiophosphate has from C₆ to C₂₄ carbon atoms; or wherein the aryl group of the zinc diaryl dithiophosphate has from C₆ to C₂₀ carbon atoms.

7. The lubricating oil composition according to Claim 1, wherein the respective ratio of zinc primary dialkyl dithiophosphate to zinc secondary dialkyl dithiophosphate is a range from 3:2 to 2:3, based on the phosphorus content; or wherein the respective ratio of zinc primary dialkyl dithiophosphate to zinc secondary dialkyl dithiophosphate is 1:1, based on the phosphorus content.

8. The lubricating oil composition according to Claim 1, wherein the respective ratio of the mixture of zinc primary dialkyl dithiophosphate and zinc secondary dialkyl dithiophosphate to zinc diaryl dithiophosphate is a range from 4:1 to 1:1, based on the phosphorus content; or wherein the respective ratio of the mixture of zinc primary dialkyl dithiophosphate and zinc secondary dialkyl dithiophosphate to zinc diaryl dithiophosphate is 2:1, based on the phosphorus content.

9. The lubricating oil composition according to Claim 1, wherein the respective ratio of the mixture of zinc primary dialkyl dithiophosphate to zinc secondary dialkyl dithiophosphate to zinc diaryl dithiophosphate is 1:1:1, based on the phosphorus content.

10. The lubricating oil composition according to Claim 1, wherein the total phosphorus content of the lubricating oil composition is less than 0.05 wt %, based on the total weight of the lubricating oil composition.

11. The lubricating oil composition according to Claim 1, wherein the total sulfur content of the lubricating oil composition is less than 0.5 wt %, based on the total weight of the lubricating oil composition; or wherein the total sulfur content of the lubricating oil composition is less than 0.2 wt %, based on the total weight of the lubricating oil composition.

12. The lubricating oil composition according to Claim 1, wherein the total sulfated ash content of the lubricating oil composition is less than 1.2 wt %, based on the total weight of the lubricating oil composition; or wherein the total sulfated ash content of the lubricating oil composition is less than 1.0 wt %, based on the total weight of the lubricating oil composition; or wherein the total sulfated ash content of the lubricating oil composition is less than 0.8 wt %, based on the total weight of the lubricating oil composition.

13. A method for improving lead corrosion, said method comprising operating an internal combustion engine with a lubricating oil composition as claimed in any preceding claim.

14. The use of a lubricating oil composition as claimed in any preceding claim for use in improving lead corrosion in operation of an internal combustion engine.

## Patentansprüche

1. Schmierölzusammensetzung, umfassend eine größere Menge Basisöl mit Schmierviskosität und eine kleinere Menge von mindestens 0,1 Gew.-% bis 1,5 Gew.-% einer Mischung aus einem primären Zink-Dialkyldithiophosphat, einem sekundären Zink-Dialkyldithiophosphat und einem Zink-Diaryldithiophosphat, wobei das jeweilige Verhältnis, auf der Basis des Phosphorgehalts, des primären Zink-Dialkyldithiophosphats zum sekundären Zink-Dialkyldithiophosphat von 2:1 bis 1:2 ist und das Verhältnis der Mischung aus primärem Zink-Dialkyldithiophosphat und sekundärem Zink-Dialkyldithiophosphat zum Zink-Diaryldithiophosphat von 6:1 bis 1:1 und wobei die Schmierölzusammensetzung weniger als 0,06 Gew.-% Gesamtphosphorgehalt hat, auf der Basis des Gesamtgewichts der Schmierölzusammensetzung.

2. Schmierölzusammensetzung gemäß Anspruch 1, wobei die kleinere Menge der Mischung aus primärem Zink-Dialkyldithiophosphat, sekundärem Zink-Dialkyldithiophosphat und Zink-Diaryldithiophosphat von 0,3 Gew.-% bis 1,2 Gew.-% ist, auf der Basis des Gesamtgewichts der Schmierölzusammensetzung; oder wobei die kleinere Menge der Mischung aus primärem Zink-Dialkyldithiophosphat, sekundärem Zink-Dialkyldithiophosphat und Zink-Diaryldithiophosphat von 0,5 Gew.-% bis 1,0 Gew.-% ist, auf der Basis des Gesamtgewichts der Schmierölzusammensetzung.

3. Schmierölzusammensetzung gemäß Anspruch 1, wobei die Mischung von 0,05 Gew.-% bis 1,2 Gew.-% primäres Zink-Dialkyldithiophosphat enthält, von 0,05 Gew.-% bis 1,2 Gew.-% sekundäres Zink-Dialkyldithiophosphat und von 0,02 Gew.-% bis 0,7 Gew.-% Zink-Diaryldithiophosphat, auf der Basis des Gesamtgewichts der Schmierölzusammensetzung; oder wobei die Mischung von 0,1 Gew.-% bis 0,7 Gew.-% primäres Zink-Dialkyldithiophosphat enthält, von 0,1 Gew.-% bis 0,7 Gew.-% sekundäres Zink-Dialkyldithiophosphat und von 0,05 Gew.-% bis 0,5 Gew.-% Zink-Diaryldithiophosphat, auf der Basis des Gesamtgewichts der Schmierölzusammensetzung; oder wobei die Mischung von 0,2 Gew.-% bis 0,5 Gew.-% primäres Zink-Dialkyldithiophosphat enthält, von 0,2 Gew.-% bis 0,5 Gew.-% sekundäres Zink-Dialkyldithiophosphat und von 0,1 Gew.-% bis 0,3 Gew.-% Zink-Diaryldithiophosphat, auf der Basis des Gesamtgewichts der Schmierölzusammensetzung.

4. Schmierölzusammensetzung gemäß Anspruch 1, wobei die primäre Alkylgruppe des primären Zink-Dialkyldithiophosphats von C₁- bis C₁₃-Kohlenstoffatome hat; oder wobei die primäre Alkylgruppe des primären Zink-Dialkyldithiophosphats von C₃- bis C₁₀-Kohlenstoffatome hat; oder wobei die primäre Alkylgruppe des primären Zink-Dialkyldithiophosphats von C₆- bis C₈-Kohlenstoffatome hat.

5. Schmierölzusammensetzung gemäß Anspruch 1, wobei die sekundäre Alkylgruppe des sekundären Zink-Dialkyldithiophosphats von C₃- bis C₁₃-Kohlenstoffatome hat; oder wobei die sekundäre Alkylgruppe des sekundären Zink-Dialkyldithiophosphats von C₃- bis C₈-Kohlenstoffatome hat; oder wobei die sekundäre Alkylgruppe des sekundären Zink-Dialkyldithiophosphats von C₃-bis C₆-Kohlenstoffatome hat.

6. Schmierölzusammensetzung gemäß Anspruch 1, wobei die Arylgruppe des Zink-Diaryldithiophosphats von C₆- bis C₃₀-Kohlenstoffatome hat; oder wobei die Arylgruppe des Zink-Diaryldithiophosphats von C₆- bis C₂₄-Kohlenstoffatome hat; oder wobei die Arylgruppe des Zink-Diaryldithiophosphats von C₆- bis C₂₀-Kohlenstoffatome hat.

7. Schmierölzusammensetzung gemäß Anspruch 1, wobei das jeweilige Verhältnis von primärem Zink-Dialkyldithiophosphat zu sekundärem Zink-Dialkyldithiophosphat in einem Bereich von 3:2 bis 2:3 ist, auf der Basis des Phosphorgehalts; oder wobei das jeweilige Verhältnis von primärem Zink-Dialkyldithiophosphat zu sekundärem Zink-Dialkyldithiophosphat 1:1 ist, auf der Basis des Phosphorgehalts.

8. Schmierölzusammensetzung gemäß Anspruch 1, wobei das jeweilige Verhältnis der Mischung aus primärem Zink-Dialkyldithiophosphat und sekundärem Zink-Dialkyldithiophosphat zu Zink-Diaryldithiophosphat im Bereich von 4:1 bis 1:1 ist, auf der Basis des Phosphorgehalts; oder wobei das jeweilige Verhältnis der Mischung aus primärem Zink-Dialkyldithiophosphat und sekundärem Zink-Dialkyldithiophosphat zu Zink-Diaryldithiophosphat 2:1 ist, auf der Basis des Phosphorgehalts.

9. Schmierölzusammensetzung gemäß Anspruch 1, wobei das jeweilige Verhältnis der Mischung aus primärem Zink-Dialkyldithiophosphat zu sekundärem Zink-Dialkyldithiophosphat zu Zink-Diaryldithiophosphat 1:1:1 ist, auf der Basis des Phosphorgehalts.

10. Schmierölzusammensetzung gemäß Anspruch 1, wobei der Gesamtphosphorgehalt der Schmierölzusammensetzung weniger als 0,05 Gew.-% ist, auf der Basis des Gesamtgewichts der Schmierölzusammensetzung.

11. Schmierölzusammensetzung gemäß Anspruch 1, wobei der Gesamtschwefelgehalt der Schmierölzusammensetzung weniger als 0,5 Gew.-% ist, auf der Basis des Gesamtgewichts der Schmierölzusammensetzung; oder wobei der Gesamtschwefelgehalt der Schmierölzusammensetzung weniger als 0,2 Gew.-% ist, auf der Basis des Gesamtgewichts der Schmierölzusammensetzung.

12. Schmierölzusammensetzung gemäß Anspruch 1, wobei der Gesamtsulfataschegehalt der Schmierölzusammensetzung weniger als 1,2 Gew.-% ist, auf der Basis des Gesamtgewichts der Schmierölzusammensetzung; oder wobei der Gesamtsulfataschegehalt der Schmierölzusammensetzung weniger als 1,0 Gew.-% ist, auf der Basis des Gesamtgewichts der Schmierölzusammensetzung; oder wobei der Gesamtsulfataschegehalt der Schmierölzusammensetzung weniger als 0,8 Gew.-% ist, auf der Basis des Gesamtgewichts der Schmierölzusammensetzung.

13. Verfahren zum Verbessern von Bleikorrosion, das Verfahren umfassend Betreiben eines Verbrennungsmotors mit einer Schmierölzusammensetzung aus irgendeinem vorhergehenden Anspruch.

14. Verwendung einer Schmierölzusammensetzung aus irgendeinem vorhergehenden Anspruch zur Verwendung zum Verbessern von Bleikorrosion bei Betrieb eines Verbrennungsmotors.

## Revendications

1. Composition d'huile lubrifiante comprenant une quantité majeure d'huile de base de viscosité lubrifiante et une quantité mineure d'au moins 0,1 pour cent en poids à 1,5 pour cent en poids d'un mélange d'un dialkyledithiophosphate primaire de zinc, d'un dialkyledithiophosphate secondaire de zinc et d'un diaryledithiophosphate de zinc, où le rapport respectif, sur la base du contenu en phosphore, entre le dialkyledithiophosphate primaire de zinc et le dialkyledithiophosphate secondaire de zinc est entre 2:1 et 1:2, et le rapport entre le mélange du dialkyledithiophosphate primaire de zinc et du dialkyledithiophosphate secondaire de zinc et le diaryledithiophosphate de zinc est entre 6:1 et 1:1, et où la composition d'huile lubrifiante a moins de 0,06 pour cent en poids de contenu total en phosphore, sur la base du poids total de la composition d'huile lubrifiante.

2. Composition d'huile lubrifiante selon la revendication 1, dans laquelle la quantité mineure du mélange d'un dialkyledithiophosphate primaire de zinc, d'un dialkyledithiophosphate secondaire de zinc et d'un diaryledithiophosphate de zinc est entre 0,3 pour cent en poids et 1,2 pour cent en poids, sur la base du poids total de la composition d'huile lubrifiante ; ou dans laquelle la quantité mineure du mélange d'un dialkyledithiophosphate primaire de zinc, d'un dialkyledithiophosphate secondaire de zinc et d'un diaryledithiophosphate de zinc est entre 0,5 pour cent en poids et 1,0 pour cent en poids, sur la base du poids total de la composition d'huile lubrifiante.

3. Composition d'huile lubrifiante selon la revendication 1, dans laquelle le mélange contient entre 0,05 pour cent en poids et 1,2 pour cent en poids d'un dialkyledithiophosphate primaire de zinc, entre 0,05 pour cent en poids et 1,2 pour cent en poids d'un dialkyledithiophosphate secondaire de zinc et entre 0,02 pour cent en poids et 0,7 pour cent en poids d'un diaryledithiophosphate de zinc, sur la base du poids total de la composition d'huile lubrifiante ; ou dans laquelle le mélange contient entre 0,1 pour cent en poids et 0,7 pour cent en poids d'un dialkyledithiophosphate primaire de zinc, entre 0,1 pour cent en poids et 0,7 pour cent en poids d'un dialkyledithiophosphate secondaire de zinc et entre 0,05 pour cent en poids et 0,5 pour cent en poids d'un diaryledithiophosphate de zinc, sur la base du poids total de la composition d'huile lubrifian-telubrifiante ; ou dans laquelle le mélange contient entre 0,2 pour cent en poids et 0,5 pour cent en poids d'un dialkyledithiophosphate primaire de zinc, entre 0,2 pour cent en poids et 0,5 pour cent en poids d'un dialkyledithiophosphate secondaire de zinc et entre 0,1 pour cent en poids et 0,3 pour cent en poids d'un diaryledithiophosphate de zinc, sur la base du poids total de la composition d'huile lubrifiante.

4. Composition d'huile lubrifiante selon la revendication 1, dans laquelle le groupement alkyle primaire du dialkyledithiophosphate primaire de zinc a entre C₁ et C₁₃ atomes de carbone ; ou dans laquelle le groupement alkyle primaire du dialkyledithiophosphate primaire de zinc a entre C₃ et C₁₀ atomes de carbone ; ou dans laquelle le groupement alkyle primaire du dialkyledithiophosphate primaire de zinc a entre C₆ et C₈ atomes de carbone.

5. Composition d'huile lubrifiante selon la revendication 1, dans laquelle le groupement alkyle secondaire du dialkyledithiophosphate secondaire de zinc a entre C₃ et C₁₃ atomes de carbone ; ou dans laquelle le groupement alkyle secondaire du dialkyledithiophosphate secondaire de zinc a entre C₃ et C₈ atomes de carbone ; ou dans laquelle le groupement alkyle secondaire du dialkyledithiophosphate secondaire de zinc a entre C₃ et C₆ atomes de carbone.

6. Composition d'huile lubrifiante selon la revendication 1, dans laquelle le groupement aryle du diaryledithiophosphate de zinc a entre C₆ et C₃₀ atomes de carbone ; ou dans laquelle le groupement aryle secondaire du diaryledithiophosphate de zinc a entre C₆ et C₂₄ atomes de carbone ; ou dans laquelle le groupement alryle du diaryledithiophosphate de zinc a entre C₆ et C₂₀ atomes de carbone.

7. Composition d'huile lubrifiante selon la revendication 1, dans laquelle le rapport respectif entre le dialkyledithiophosphate primaire de zinc et le dialkyledithiophosphate secondaire de zinc est dans l'intervalle de 3:2 à 2:3, sur la base de la teneur en phosphore ; ou dans laquelle le rapport respectif entre le dialkyledithiophosphate primaire de zinc et le dialkyledithiophosphate secondaire de zinc est 1:1, sur la base de la teneur en phosphore.

8. Composition d'huile lubrifiante selon la revendication 1, dans laquelle le rapport respectif entre le mélange du dialkyledithiophosphate primaire de zinc et du dialkyledithiophosphate secondaire de zinc par rapport au diaryledithiophosphate de zinc est dans l'intervalle de 4:1 à 1:1, sur la base de la teneur en phosphore ; ou, dans laquelle le rapport respectif entre le mélange du dialkyledithiophosphate primaire de zinc et du dialkyledithiophosphate secondaire de zinc et le diaryledithiophosphate de zinc est 2:1, sur la base de la teneur en phosphore.

9. Composition d'huile lubrifiante selon la revendication 1, dans laquelle le rapport respectif du mélange entre le dialkyledithiophosphate primaire de zinc, le dialkyledithiophosphate secondaire de zinc et le diaryledithiophosphate de zinc est 1:1:1, sur la base de la teneur en phosphore.

10. Composition d'huile lubrifiante selon la revendication 1, dans laquelle la teneur totale en phosphore de la composition d'huile lubrifiante est moins de 0,05 pour cent en poids, sur la base du poids total de la composition d'huile lubrifiante.

11. Composition d'huile lubrifiante selon la revendication 1, dans laquelle la teneur totale en soufre de la composition d'huile lubrifiante est moins de 0,5 pour cent en poids, sur la base du poids total de la composition d'huile lubrifiante ; ou dans laquelle la teneur totale en soufre de la composition d'huile lubrifiante est moins de 0,2 pour cent en poids, sur la base du poids total de la composition d'huile lubrifiante.

12. Composition d'huile lubrifiante selon la revendication 1, dans laquelle la teneur totale en cendres sulfatées de la composition d'huile lubrifiante est moins de 1,2 pour cent en poids, sur la base du poids total de la composition d'huile lubrifiante ; ou dans laquelle la teneur totale en cendres sulfatées de la composition d'huile lubrifiante est moins de 1,0 pour cent en poids, sur la base du poids total de la composition d'huile lubrifiante ; ou dans laquelle la teneur totale en cendres sulfatées de la composition d'huile lubrifiante est moins de 0,8 pour cent en poids, sur la base du poids total de la composition d'huile lubrifiante.

13. Procédé pour améliorer la corrosion du plomb, ledit procédé comprenant opérer un moteur à combustion interne avec une composition d'huile lubrifiante comme revendiquée dans l'une quelconque revendication précédente.

14. Utilisation d'une composition d'huile lubrifiante comme revendiquée dans l'une quelconque revendication précédente pour l'utilisation pour améliorer la corrosion du plomb lors de l'opération d'un moteur à combustion interne.
